

## UNITED STATES PATENT OFFICE

2,006,565

## MAGNESIUM BASE ALLOY

Robert T. Wood, Cleveland, Ohio, assignor, by  
mesne assignments, to Magnesium Develop-  
ment Corporation, a corporation of Delaware

No Drawing. Application May 18, 1934,  
Serial No. 726,317

## 3 Claims. (Cl. 75—1)

This invention relates to magnesium base alloys and it is especially concerned with an improvement in alloys designed for hot working.

Magnesium base alloys have been extensively used for castings but considerable difficulty has been experienced in hot working alloys of this type. Magnesium base alloys generally possess a low ductility at hot working temperatures and consequently develop internal ruptures very easily as well as external cracks. Such breaks in the continuity of the alloy structure are not healed by subsequent working with the result that the worked article must be discarded. Even the most careful heating and handling of the alloy in hot working operations fails to remedy this condition. It is moreover often desirable to use a wrought article for a given application because of the greater uniformity of structure and higher mechanical properties that are attainable as compared to similar properties of a cast product. It has been particularly difficult to hot form magnesium base alloys into intricate shapes which has necessitated the substitution of other materials at the sacrifice of saving in weight.

It is an object of my invention to provide magnesium base alloys that can be readily hot worked without developing internal or external breaks in the structure. Another object is to produce an alloy that is sufficiently plastic at hot working temperatures to permit successful formation of intricate shapes on a commercial scale.

My invention is predicated upon the discovery that a magnesium base alloy composed of from about 1.0 to 15 per cent of tin, 0.1 to 3 per cent of manganese and 0.1 to 1.0 per cent of silicon, has the aforementioned properties. While the favorable hot working quality of the alloy is manifest over the entire range of composition indicated, I have found that in general the most satisfactory combination of working properties and strength is present in alloys containing from about 4 to 10

per cent of tin, 0.5 to 1.5 per cent of manganese and 0.2 to 1 per cent of silicon.

A preferred alloy coming within the last mentioned range is one containing about 6 per cent of tin, 1 per cent of manganese and 0.5 per cent of silicon. This alloy forges very well and is adapted to the making of wrought shapes which have hitherto been very difficult to form. In the forged condition the alloy has a tensile strength of about 34,000 lbs. per sq. in., a yield strength of about 21,000 lbs. per sq. in., and an elongation of about 4 per cent in two inches.

The hot working operations on magnesium base alloys have usually been conducted between the temperatures of about 500 and 800° F. but with my improved alloy it is possible to heat the work up to as high as 950° F. without danger of "hot shortness". The higher temperature aids in giving greater plasticity to the alloy, as well as the nature of the alloying constituents.

The alloys herein disclosed respond to the usual thermal treatments employed in the art to improve the mechanical properties of magnesium base alloys.

The term magnesium base alloy as used hereinabove and in the appended claims refers to those alloys containing 50 per cent or more of magnesium.

## I claim:

1. A magnesium base alloy composed of from about 1 to 15 per cent of tin, 0.1 to 3.0 per cent of manganese, and 0.1 to 1.0 per cent of silicon, the balance magnesium.

2. A magnesium base alloy composed of from about 4 to 10 per cent of tin, 0.5 to 1.5 per cent of manganese and 0.2 to 1 per cent of silicon, the balance magnesium.

3. A magnesium base alloy consisting of about 6 per cent of tin, 1 per cent of manganese and 0.5 per cent of silicon, the balance magnesium.

ROBERT T. WOOD.